

Patented Sept. 5, 1922.

1,428,087

# UNITED STATES PATENT OFFICE.

JAMES H. GRAVELL, OF ELKINS PARK, PENNSYLVANIA.

## RUST-RESISTING STEEL AND METHOD OF PRODUCING SAME.

No Drawing.

Application filed June 22, 1921. Serial No. 479,683.

To all whom it may concern:

Be it known that I, JAMES H. GRAVELL, a citizen of the United States, residing at Elkins Park, in the county of Montgomery and State of Pennsylvania, have invented a new and useful Improvement in Rust-Resisting Steel and Methods of Producing Same, of which the following is a specification.

This invention relates to iron and steel and it is particularly directed to rust resisting steel.

The object of the invention is to provide rolled steel that rusts with difficulty or is not so liable to rust as ordinary rolled steel found on the market at the present time.

According to the present methods of making rolled steel and iron, the steel billet is heated to a high temperature and rolled to the desired shape. This produces the hot rolled steel of commerce which is covered with a substantial coating of oxide which causes it to look black. If a metallic or bright finish is required, the hot rolled steel is pickled with an acid to remove the oxide and then rolled or drawn cold to secure the high finish. The term "rolling" will be used to include "drawing." If a thin plate or strip is required, it may be processed several times. Between the cold rollings the metal is annealed during which great care is exercised to prevent the air from contacting with the metal while it is heated, as otherwise it would be oxidized and would have to be again pickled to remove the oxide or scale.

Steel produced by these methods rusts rapidly while stored or being shipped. It is natural for the metal to rust in the atmosphere, but the natural rusting is accelerated by the presence of impurities received in the pickling operation, such for instance as sulfuric and other acids and salts.

I have discovered that if a thin coating of iron phosphate is given to the metal before rolling and that if this coating is rolled onto or into the surface in the rolling operation, the rust accelerators are neutralized and the natural rusting tendencies of the metal are greatly reduced. Metals treated according to my process are distinguished from other metals by a darker looking surface and by their freedom from rusting, and they may be shipped or stored for long periods without danger of rusting although

not protected by a coating of oil which is now the universal custom.

To process the metal according to my invention, it may be first hot rolled and then freed of its oxidized surface by any of the well known methods, such as "etching" and sand-blasting or sudden chilling and it may be washed. It is then given a coating of iron phosphate. This may be done by boiling the metal in a dilute solution of phosphoric acid (one pound of absolute acid to 100 pounds of water) or the metal may be simply dipped in a solution of phosphoric acid and water (one pound of acid to 20 pounds of water). The water may be hot or cold. Another method of forming the phosphate coating on the surface is to apply a coating of a thermally decomposable phosphate such as ammonium or aniline phosphate and to then heat the metal to liberate phosphoric acid which attacks the surface forming the phosphate coating. Or an acid salt of phosphoric acid may be applied to the surface which will have sufficient acid reaction to produce the desired coating.

After securing the phosphated surface, the metal is then rolled. It may be allowed to thoroughly dry first if the wet methods mentioned above have been used or the metal may be passed through the rolls in the wet condition.

The metal resulting from this process is dull in appearance and has the advantageous property of not readily rusting and it may be painted without danger of the metal rusting under the paint as the cause for this is neutralized in my process by the action of the free or combined phosphoric acid.

It will be obvious to those skilled in the art that modifications may be made in details of procedure and in its chemical aspects the range of equivalents is wide, hence I do not intend to limit the invention as to such matters or otherwise than as the prior art and the appended claims may require.

I claim:

1. The method of producing rust resisting steel consisting in treating the steel with phosphoric acid and then rolling the steel.
2. The method of producing rust resisting steel consisting in pickling the steel, then treating the steel with phosphoric acid, and then rolling the steel.
3. The method of producing rust resist-

ing steel consisting in pickling the steel, washing the steel to remove the pickle, then treating the steel with phosphoric acid, and then rolling the steel.

5 4. The method of producing rust resisting steel consisting in forming a coating of iron phosphate on the surface of the steel and then rolling the steel.

5. The method of treating steel to prevent 10 it from rusting which consists in rolling into

its surface a rust inhibitive coating developed from the steel, substantially as described.

6. A new article of manufacture consisting of a body of steel having a pressed-in 15 surface of phosphate.

7. A new article of manufacture consisting of a body of steel having a pressed-in surface of iron phosphate.

JAMES H. GRAVELL.